

Nov. 30, 1926.

1,608,866

N. L. SNOW ET AL

BOILER CLEANER

Filed June 14, 1926

2 Sheets-Sheet 1



Inventors  
Norman L. Snow  
Samuel F. Cox

Whittmore Hubert Whittmore

H. C. Cheney

Attorneys

Nov. 30, 1926.

1,608,866

N. L. SNOW ET AL

BOILER CLEANER

Filed June 14, 1926

2 Sheets-Sheet 2

*Fig. 2.*



*Fig. 5*

*Fig. 6*



*Fig. 3.*

*Fig. 4*



Inventors

Norman L. Snow  
Samuel E. Cox

By

Whittmore, Hubert Whittmore

Belknap

Attorneys

## UNITED STATES PATENT OFFICE.

NORMAN L. SNOW AND SAMUEL F. COX, OF DETROIT, MICHIGAN, ASSIGNEES TO DIAMOND POWER SPECIALTY CORPORATION, OF DETROIT, MICHIGAN, A CORPORATION OF MICHIGAN.

## BOILER CLEANER.

Application filed June 14, 1926. Serial No. 115,972.

The invention relates to boiler cleaners and refers more particularly to an improved blower element.

We have discovered that a soot blower element when made of an iron chromium alloy of the proportions hereinafter pointed out, has certain highly desirable characteristics not found in soot blower elements as heretofore made.

10 We have found that when a soot blower element is made of the alloy referred to, it can readily be formed into tubes with relatively thin walls, which tubes possess to such a degree that desirable combination 15 of physical properties, which we may best describe as toughness, that they will not be ruptured by sudden changes in temperature, caused by the contact of the cleaning fluid, such as steam, with the tube when the latter 20 is highly heated. We have found moreover, that such a tube will stand up satisfactorily under the operating conditions of a modern boiler where soot blower elements 25 are subjected to very high temperatures in the presence of oxygen and the other furnace gases together with the furnace ash containing as it ordinarily does, iron oxides, alumina, silica, lime and magnesia; such an alloy soot blower element resists 30 the erosive action of said high temperature furnace gases which frequently impinge against the element with considerable high velocity carrying with them quantities of the said furnace ash. We have further found that a soot blower element made of such an alloy will not sag unduly between the supports provided for it in the boiler, even though the blower tube be heated to a bright red or somewhat greater heat and 40 though the supports be relatively widely spaced.

We have further found that our alloy possesses such properties that as before pointed out, it may be readily formed into tubes, such processes being preferably carried out by the application of mechanical force.

Referring to the accompanying drawings

in which like reference characters indicate corresponding parts:

50 Figure 1 represents a section through a typical boiler showing our blower element associated therewith;

Figure 1<sup>a</sup> is a sectional view along 1<sup>a</sup>—1<sup>a</sup> of Figure 1;

55 Figure 2 is a view of our blower tube constructed in accordance with one embodiment of our invention;

Figure 3 is a like view of a portion of our blower tube constructed in accordance 60 with a modified form of our invention;

Figure 4 is a sectional view of the same along the line 4—4 of Figure 3;

Figure 5 is a view of our blower element 65 corresponding to Figures 2 and 3 but illustrating a further and preferred modified form of our invention, and

Figure 6 is a sectional view of the same along the line 6—6 of Figure 5.

70 Referring to the drawings, reference character A represents a boiler of any suitable type and construction having the usual boiler tubes 10. Mounted at any suitable point or points in the boiler are the soot blower tubes or elements B, one of which for purposes of illustration is shown mounted for rotation in the head 11, cleaning fluid such as steam, air, etc. being supplied through pipe 12 to the blower element. If desired the elements may be supported at suitable 75 intervals along their length by the supporting bearings 13. The manner of supporting the elements forms no feature of our invention, and the elements may or may not be mounted for rotation as desired.

85 The blower element constructed in accordance with our invention is formed of iron with chromium as the principal alloying ingredient, the chromium content ranging from 11 to 30 per cent, the upper limit 90 being determined principally by considerations of working the material by the application of mechanical force. We have found, for example, that the preferred specific quantities of chromium throughout the aforesaid range may be divided into

three "groups" which for convenience of group does not lend itself as readily to this discussion may be termed as the "low chromium group", the "intermediate chromium group" and the "high chromium group".

5 The specific analyses of the alloy material comprising these groups may conveniently be as follows:—

*Low chromium group.*

|                                         | Per cent. |
|-----------------------------------------|-----------|
| 10 Chromium                             | 11 to 14  |
| Carbon less than .50%, preferably under | .25       |
| Silicon less than                       | .50       |
| 15 Manganese less than                  | .50       |
| Sulphur less than                       | .045      |
| Phosphorus less than                    | .045      |
| Iron balance.                           |           |

*Intermediate chromium group.*

|                                               | Per cent.   |
|-----------------------------------------------|-------------|
| 20 Chromium                                   | 16 to 19    |
| Carbon less than .25%, preferably under       | .10         |
| 25 Silicon .5 to 2.0%, preferably .75 to 1.25 | .75 to 1.25 |
| Manganese less than                           | .50         |
| Sulphur less than                             | .045        |
| Phosphorus less than                          | .045        |
| Iron balance.                                 |             |

*High chromium group.*

|                                            | Per cent. |
|--------------------------------------------|-----------|
| 30 Chromium 26 to 30%, preferably 26 to 28 | 26 to 28  |
| Carbon less than .50%, preferably under    | .25       |
| 35 Silicon less than                       | .50       |
| Manganese less than                        | .50       |
| Sulphur less than                          | .045      |
| Phosphorus less than                       | .045      |
| Iron balance.                              |           |

40 In each of the aforesaid groups, representing typical illustrative analyses, the silicon, manganese, sulphur, and phosphorus while not being strictly essential to the material 45 are generally present in the amounts stated following the general practice of good open hearth steel as used in the manufacture of boiler tubes. Obviously, relatively small amounts of various chemical elements may 50 enter into composition of the material, other than the elements stated, without departing from the salient features of our invention. For example, nickel in small amounts as 55 from 2 to 3% may be added to facilitate working the material.

The alloy material in the ranges of the low and intermediate chromium groups may conveniently be formed into blower tubes by the seamless method as in the ordinary 60 method of manufacturing seamless boiler tubes or the like consisting essentially in forcing a heated bar of the material over a piercing point. A seamless soot blower element constructed by such a method is 65 shown in Figure 2. The high chromium

method as do the aforesaid low and intermediate chromium groups.

In forming the blower elements from our alloy material of the high chromium group 70 which group we have found affords the best results in service, we might form the blower element as shown in Figures 3 and 4. In this instance the element B is formed from the alloy material in relatively thin rolled strip, formed as by the usual rolling mill method, the strip being then wound or coiled spirally with the connecting edges of the strip preferably slightly overlapped to accommodate suitable fasteners such as rivets 80 14. Obviously, if desired, the alloy material in the low and intermediate chromium groups, as well as throughout the entire chromium range as aforesaid, might also be formed in this manner.

85 Referring to Figures 5 and 6, we have illustrated a further modified blower element B adapted principally to the use of the material of the high chromium group, although adaptable to use of our material containing chromium in percentages throughout the entire aforesaid range. In this embodiment, which is preferred for alloys of the high chromium group, the alloy material may be formed in strip form as aforesaid and rolled into substantially tubular shape, the connecting edges being permanently joined as by welding at 15. Material of this nature in relatively thin rolled form can be welded quite satisfactory as distinguished from the relatively thick wall heavy cast element sections which can be satisfactory welded only with the greatest difficulty.

90 The various forms of blower elements may be provided with nozzles 16 for discharging the cleaning fluid adjacent the parts of the boiler to be cleaned. Such nozzles may be formed of our alloy and fixed in the element in any preferred manner.

95 If desired blower elements may be formed by the application of mechanical force in various other methods from those illustrated without departing from the salient features of our invention. For example, the connecting edges of the spirally formed element shown in Figures 3 and 4 may, if desired, be welded instead of fastened by rivets; or the connecting edges of the element shown in Figures 5 and 6 may be overlapped and connected by rivets; other modifications will readily suggest themselves, and we do not limit our invention to the specific embodiment shown except as specifically recited in our claims.

100 What we claim as our invention is:

1. A soot blower cleaner tube adapted in its normal operation to be subjected to the destructive agencies set into action by the 105 operation of the boiler to which the tube is 110 115 120 125 130 135

applied and to be subjected to sudden temperature changes occasioned by the passage of relatively cool cleaning fluid through the tube while the tube is highly heated, said tube being wrought from alloy material containing chromium as the principal alloying element in sufficient quantity to resist the aforesaid destructive agencies, said alloy having the further characteristic of resisting disruption when subjected to the aforesaid temperature changes.

2. A soot blower cleaner tube adapted in its normal operation to be subjected to the destructive agencies set into action by the operation of the boiler to which the tube is applied and to be subjected to sudden temperature changes occasioned by the passage of relatively cool cleaning fluid through the tube while the tube is highly heated, said tube being wrought from alloy material containing at least approximately 16% chromium to resist the aforesaid destructive

agencies, said alloy having the further characteristic of resisting disruption when subjected to the aforesaid temperature changes. 25

3. A soot blower cleaner tube adapted in its normal operation to be subjected to the destructive agencies set into action by the operation of the boiler to which the tube is applied and to be subjected to sudden temperature changes occasioned by the passage of relatively cool cleaning fluid through the tube while the tube is highly heated, said tube being wrought from alloy material containing in excess of approximately 25% 30 chromium to resist the aforesaid destructive agencies, said alloy having the further characteristic of resisting disruption when subjected to the aforesaid temperature changes. 35

In testimony whereof we affix our signatures. 40

NORMAN L. SNOW.  
SAMUEL F. COX.